

## UNITED STATES PATENT OFFICE

GEORGE W. BENNETT, OF CINCINNATI, OHIO

## COMPOSITION AND PROCESS FOR RUBBER BLANKET PRINTING

No Drawing.

Application filed September 5, 1930. Serial No. 480,025.

The present invention relates to improvements in printing with blankets, for example printing on offset printing presses, or the like, or printing in any kind of a process where a printer's blanket is employed. The offset press will be discussed in connection with the invention, this being a well known type of press used in the printing industry. In the ordinary process of printing with an offset press, the type, or an engraved or etched plate or the like, is first brought into contact, while mounted on a roller, with an inked roller, in order to ink the face of the type or the desired portions of the engraved or etched plate. During the rotation of the roll, carrying the type, the face of the type comes into contact with a rubber blanket mounted on a roller, leaving ink on the said rubber blanket, the roller carrying the blanket then revolves further and a sheet of paper passes between the blanket roll and a pressure roll, in order to transfer the ink from the rubber blanket onto the paper. The roller carrying the type and the roller carrying the blanket must of course rotate at exactly the same speed, but in opposite directions. The face of the inking roller should travel at the same speed as the face of the type roller, and the face of the pressure roller should travel at the same speed as the face of the blanket roller, although the pressure roller and inking roller may be of a larger or smaller size than the type roller and blanket roller.

A skilled printer or pressman will readily understand what is meant by the term "make ready". Briefly, it is that operation involving the building up or patching a packing with "folio" or similar thin transparent paper at those portions where a faint impression or perhaps, where there is no impression, whatever and also cutting out those portions where the impression is too great, with the final result that an even impression is obtained over all portions of the printing surface. This packing is placed under the rubber on the cylinder and often constitutes several sheets of paper carrying patches. This "make ready" operation when performed in the ordinary manner is very time consuming and in printing jobs involving "cuts", very

often requires 10 to 18 hours to "make ready".

In practicing my invention, it is possible to greatly reduce the time required for "making ready", because I merely apply a composition to the rubber on the printing cylinder whereby all cavities and depressions are filled in and hence, I avoid the usual steps of "marking out" a trial sheet and patching with "folio". This composition which is hereafter described should be applied to the printing blanket preferably about a day before the printing blanket is placed on the cylinder of the press. The time during which the blanket is allowed to stand after treatment with my novel composition will of course vary with the condition of the rubber and I have found that where a rubber is in good condition one hour is sufficient and I have also found that in extreme cases it is necessary to allow the blanket to stand for a period of one week before it can be used on the cylinder press.

On account of various defects, the surface of the rubber blanket may become injured or "mashed" and this may for example be produced by a sheet of paper getting wrinkled and then passing in a wrinkled condition between the blanket roller and the pressure roller. Heretofore when mashing of the blanket has occurred, it has usually been necessary to disconnect one end of the blanket, after stopping the press, and then build up with small carefully cut out pieces of paper, one or several thicknesses, on the back or fabric side of the blanket, to build up the desired thickness since the face of the blanket roll must be true, in order to produce satisfactory printing. This patching of the blanket requires much time, particularly when the mashes are bad or are uneven. In common practice, after patching has been resorted to, and the blanket fastened again onto the roller, the usual practice has been to wash the face of the blanket with benzine, for example with a sponge or the like, in order to remove all ink, dried ink and the like, and to then powder the surface with finely powdered sulphur, or with a mixture of finely powdered sulphur and finely powdered French chalk (talc).

A further objection to blanket printing is that sometimes the blanket becomes embossed.

This embossing may be produced by certain special inks which carry considerable amount of oil particularly drying oils, and by overpacking (producing extra pressure) and various other ways. After a particular printing job has been completed, or when the embossing gets too bad, the usual practice has been to remove and discard the printer's blanket from the roll.

10 From the above causes and from the other causes, which cause injury and deterioration of the printer's blanket, a blanket has a useful life period varying from one day to three months, but it may be stated that the average useful life period of a blanket is ordinarily 15 about two months.

20 In accordance with the present invention, I have found that small mashes which are not very deep, on the rubber surface of the blanket can readily be overcome by the use of a single 25 application of a composition as herein described, whereas deeper or larger mashes can readily be overcome by applying the composition to both the front and the back of the 30 blanket, the application to the blanket of the composition in question being much more expeditious than the paper packing heretofore usually resorted to.

The composition preferably employed is 35 made up as follows:

|                                                    |                |
|----------------------------------------------------|----------------|
| Kerosene                                           | 1 ounce        |
| Spirits of turpentine                              | 1 ounce        |
| "Penetrating oil" largely composed of hydrocarbons | 1 ounce        |
| Oil of sassafras                                   | 0.5 ounce      |
| Oil of cloves                                      | 0.5 ounce      |
| Powdered sulphur                                   | 1 teaspoonful  |
| Powdered orris root                                | 2 teaspoonfuls |

40 together with any suitable color. The color is for example Prussian blue ground in a drying oil or mixture of drying oil and japan drier.

45 The hydrocarbon oil used in the "penetrating oil" may be kerosene or similar distillate of petroleum, mixed with say an equal amount of coal tar creosote, this being very satisfactory for the purpose, although other 50 penetrating oils can be employed.

In place of kerosene, the first mentioned ingredient of the composition, I may use other relatively light petroleum distillates, preferably less volatile than gasoline and preferably more volatile than spindle oil.

60 The oil of sassafras and oil of cloves impart a pleasant odor to the oil mixture but they also have an important function of swelling the rubber and penetrating the rubber readily, and these also penetrate and swell the fabric face when applied to the back of the blanket.

65 It is to be understood that before applying the above composition to the face of the 70 blanket, either the whole face of the blanket

or the portion thereof carrying the mashes are first washed with benzine, in order to remove the ink therefrom. Small mashes which are on the surface of the rubber blanket will ordinarily be cured simply by applying the above mentioned composition on the rubber surface, whereas larger or deeper mashes are preferably treated first on the surface and then on the back of the blanket (fabric side). For application either to the front or back 75 of the blanket, a small quantity of the liquid material, say on a sponge or wad of cotton is simply rubbed upon the blanket, and the composition is then allowed to dry, which requires only a few minutes. The finely powdered sulphur or a mixture of the same with finely powdered talc is then applied to the surface as above indicated, the blanket then locked back upon the roller in the customary manner and the printing at once continued 80 with. While ordinary patching may require a good deal of time, mashes can be cured according to the present invention in a small fraction only of the time required by the method heretofore commonly used.

85 Where the blanket has become embossed, as above referred to, it is only necessary to apply the composition of the present case, on and around the embossed portion of the blanket, this being also preferably done after 90 first washing with benzine. After drying, the coating of fine sulphur is applied as above referred to.

95 In accordance with the present invention it has been found that the same blanket can be 100 used for a month or even several months, in place of a few days as has been the custom heretofore.

105 In the case of rubber blankets which have become embossed it may be sufficient to apply this composition on the face side of the blanket or in some cases it is advisable to apply it on the face side and on the back both. This is done primarily for the softening effect upon the embossed portion of the rubber. 110 Treatment on embossed blankets may result only in a temporary elimination of the embossing effect, which may come back after a time, sometimes after several hours or after a day or more. In the case of the 115 mashes however the treatment as described herein cures the mashes so that they are permanently cured and do not reappear on continuation of the use of the blanket.

120 It can be seen from the foregoing that my process is applicable not only to "making ready" a blanket or matrix in the first instance but is also applicable in the repair of damaged blankets or matrices.

125 I claim:

1. A composition of matter adapted for being applied to the face side or rear side of rubber printing blankets, the same being a liquid containing as a vehicle, a liquid mineral oil product less volatile than gasoline 130

and more volatile than spindle oil, spirits of turpentine, a penetrating oil consisting largely of hydrocarbons, oil of sassafras and oil of cloves, such vehicle carrying small amounts of powdered sulphur and powdered orris root.

2. A composition of matter adapted for being applied to the face side or rear side of rubber printing blankets, the same being a liquid containing as a vehicle, a liquid mineral oil product less volatile than gasoline and more volatile than spindle oil, spirits of turpentine, a penetrating oil consisting largely of hydrocarbons, oil of sassafras and oil of cloves, such vehicle carrying small amounts of powdered sulphur and powdered orris root, together with a pigment ground in a readily drying oil.

3. A liquid mass comprising the following materials in approximately the proportions stated, namely,

|                                            |                |     |
|--------------------------------------------|----------------|-----|
| Kerosene oil                               | 1 ounce        | 75  |
| Spirits of turpentine                      | 1 ounce        | 80  |
| 25 "Penetrating oil", largely hydrocarbons | 1 ounce        | 85  |
| Oil of sassafras                           | 0.5 ounce      | 90  |
| Oil of cloves                              | 0.5 ounce      | 95  |
| Powdered sulphur                           | 1 teaspoonful  | 100 |
| 30 Powdered orris root                     | 2 teaspoonfuls | 105 |

and color in a drying oil, to give a color.

4. A process which comprises applying to the face side of rubber printing blankets, a liquid flowable composition comprising hydrocarbon oil of a gravity intermediate the gravities of gasoline and spindle oil, spirits of turpentine, "penetrating oil" consisting largely of hydrocarbons, oil of sassafras and oil of cloves, and containing finely powdered sulphur and finely powdered orris root, said application being made on "mashed" portions of the blanket, and thereafter dusting with a fine solid containing sulphur.

45 5. A process as in claim 4, in which the said material is also applied to the back side of the blanket, in the vicinity of "mashes", and thereafter dusting with a fine solid containing sulphur.

50 6. A process which comprises applying on and around "mashed" portions and "embossed portions" of at least one surface of a printer's blanket, the composition set forth in claim 2, and dusting the surface with a composition containing dry sulphur.

55 7. A process which comprises applying on and around "mashed" portions and "embossed portions" of at least one surface of a printer's blanket, the composition set forth in claim 3, and dusting the surface with a composition containing dry sulphur.

60 8. A process as set forth in claim 4, as applied to new rubber printing blankets whereby the usual "make ready" operation is dispensed with.

65 9. A process as set forth in claim 4, in

which the said composition is applied to the back of a new blanket a period of time before its use on the press varying from one hour to one week whereby the usual "make ready" operation is dispensed with. 70

In testimony whereof I affix my signature.

GEORGE W. BENNETT.

75

80

85

90

95

100

105

110

115

120

125

130